# EUROPEAN PATENT SPECIFICATION

(11) **EP 0 617 742 B1**
(45) Date of publication and mention of the grant of the patent: **21.01.1998**
(21) Application number: 93922545.4
(22) Date of filing: 11.10.1993
(51) Int. Cl.: D01D 5/40, D01F 9/00

(54) **DEVICE AND PROCESS FOR THE PRODUCTION OF FIBROUS STARCH MATERIALS**
VORRICHTUNG UND VERFAHREN ZUR HERSTELLUNG VON FASERIGEM MATERIAL AUS STAERKE
DISPOSITIF ET PROCEDE DE PRODUCTION DE MATIERES FIBREUSES A BASE D'AMIDON

(30) Priority: 16.10.1992 IT TO920837
(43) Date of publication of application: 05.10.1994
(73) Proprietor: CERESTAR HOLDING B.V., NL-4551 LA Sas van Gent (NL)
(72) Inventor: BASTIOLI, Catia, I-28100 Novara (IT); CASALE, Bruno, I-28062 Cameri (IT); ZANARDI, Gino, I-28067 Pernate (IT)
(74) Representative: Wilkinson, Stephen John
(86) International application number: EP9302782
(87) International publication number: WO9409190

(56) References cited:
- GB-A- 2 258 251
- US-A- 2 988 782
- US-A- 4 205 025
- US-A- 4 243 480

## Description

The present invention refers to a device and process for production of fibrous starch materials particularly destined for use in the production of paper and cardboard.

It is known that if aqueous colloid dispersions of starch in typical concentrations of between 5 and 40% by weight of anhydrous solid, is brought into contact with non-solvents (for example a saline solution of ammonium sulphate), it coagulates forming flakes of gel. US-A-4,243,480 describes such a process. GB-A-2258251 describes a process for producing a starch pulp comprising jet cooking an aqueous starch suspension, injecting this into a primary flux of a coagulating agent to obtain the pulp and subjecting the pulp to maturing in its own mother liquors.

US Patent No. 4,205,025 describes a process for the production of fibrils used as paper pulp using film forming polymers including substantially water-soluble starches. By the term "fibrils", materials showing a hybrid morphology which is between a film and a fibre are intended. The film forming polymer is dissolved in water to form a solution which is then injected into a precipitating means, preferably an organic non-solvent, such as an alcohol or a ketone, with the application of shearing stress in order to obtain the formation of fibrils which are then renumbered more hydrophobic through subsequent treatment in an insolublising agent.

US Patent No. 4,340,442 describes a process for the formation of fibrils which, in order to improve the hydrophobic properties of the fibrils, uses starch insoluble in water having a high amylose content (50-80% by weight), which is coagulated in a saline solution, in particular ammonium sulphate. Said starch which is substantially insoluble in water, requires a stage in which it is dissolved in alkaline solution which causes problems in the coagulation stage and problems with respect to disposal of sulphates different from ammonium salts, which are formed in said stage.

US Patent No. 4,139,699 describes a process for the production of a product having starch fibre morphology, through extrusion of a colloidal starch dispersion having a high amylopectin content in a coagulating agent. In the case where a starch having a amylopectin content of less than approximately 95% is used, it is necessary to chemically modify the starch to ensure the colloidal dispersion thereof in the aqueous system or, alternatively, the starch must be dissolved in the presence of alkaline hydroxides.

The use of alkaline hydroxides, particularly sodium hydroxide, makes the industrial application of the process described difficult, in that the coagulation stage carried out using ammonium sulphate results in the production of ammonia and formation of large quantities of sodium sulphate preventing coagulation and causing problems with respect to disposal.

US Patent No. 4,243,480 describes a process that uses the product obtained according to the process described in US Patent No. 4,139,699, for the production of paper or cardboard according to conventional paper making technology. Said product has a short fibre morphology having a diameter of between 10 and 500 microns and a length of between 0.1 and 3 mm, obtained by extruding the starch dispersion via a die into a moving coagulation bath.

US Patent No. 4,853,168 describes a process of the type described in US Patent No. 4,139,699, in which the colloidal starch dispersion adapted to be extruded is obtained by cooking an aqueous starch dispersion containing the coagulating saline solution.

In the above cited patent literature and in practical experimentation, various known devices can be used in order to finely break down the starch solution or dispersion and therefore favour a close contact with the coagulating agent, such as atomization nozzles, ejectors, mixers with stirrers, spinnerets or syringes. It has however been demonstrated experimentally that the type of device used strongly influences the final coagulated product and its properties. Devices in which the starch is coagulated in highly turbulent conditions (such as ejectors) or in which there is no ordered speed profile (mixers with stirrers), do not give rise to products with a fibrous structure, but somewhat provoke a fragmentation of the starch, with formation of flat scales (rolled onto each other) or a three dimensional aggregate.

The dimensions of these non fibrous products vary with the operating conditions and influence the characteristics of them. In the production process very small particles are lost during the separation and slow down the filtering operation in that they block the cloth; if used in the production of paper, they are not retained on the flat cloth with consequential loss of starch in the paper and an increase of COD in the paper factory waste water. On the other hand, very large particles do not integrate with the cellulose matrix fibres giving rise to defects in the produced paper.

Other negative aspect, verified for fibrids obtained from the previously described processes, consists of rather high water retention and solubility values.

A further product obtained from starch by coagulation processes, but having a fibre morphology, partly reduces the above listed disadvantages in that, thanks to its fibrous structure it increases its compatibility with the cellulose fibres, reduces the water retention in that it is more easily filterable and reduces its solubility as it has a lower specific surface.

It would therefore be desirable to have a production of a product having fibre morphology, with dimension, size distribution and physical chemical properties such to be suitable for the production of paper and cardboard and in addition to be obtainable from low cost starch such as starch from maize or potato without adopting alkaline solutions of starch for the starch used.

In the light of such a purpose, the object of this invention is a process for the preparation of fibres of starch material which comprises preparing an aqueous dispersion or solution of starch material and extruding this into a solution of a saline coagulating agent characterised in that the aqueous dispersion or solution of starch material is extruded through a microporous tubular wall of a chamber circularly ringed with said microporous wall into an annular change through which the solution of coagulating agent is caused to flow whereby the contact of the flowing coagulating agent solution with the extruded starch material dispersion or solution coagulates the starch material to form a fibrous structure.

Another object of the invention is a fibre making device characterised by the fact that it comprises:
- a tubular body comprising first means of entry for feeding the flux of starch material,
- a feeding chamber for the starch material connecting the said first means of entry,
- an annular outlet chamber of the starch material,
- a tubular element with porous walls coaxially arranged with said outlet chamber and interposed between this and the feeding chamber, adapt to extrude through the said porous walls in the said outlet chamber a variety of threads of starch material forming a envelope around the said tubular element,
- a second means of entry connecting the outlet chamber for feeding the coagulating agent flow and
- means of discharge arranged downstream from the annular outlet chamber.

It has been found that by using the process and device of the present invention it is possible to obtain a product which shows a shape ratio having a particularly narrow size distribution and centred in the range of 75-100 microns and having a water solubility, determined by the "Anthrone Test" further described later, of less than about 2% and a low water retention. Other advantages and characteristics of the process, device and product obtained according to the present invention will be further illustrated in detail in the following with reference to the enclosed drawings in which:
- figure 1 shows illustrates a flow chart of the plant for carrying out the process,
- figure 2 shows a cross section view of the fibre making device according to the invention,
- figure 3 shows a cross section view of another embodiment of the fibre making device, and
- figure 4 is an enlarged detail of a part of figures 2 and 3

With reference to the drawing in figure 1, 1 indicates a stirred dispersion for the preparation of the starch suspension in water with a dry weight typically from 5 to 50% by weight and preferably 10-40% by weight. The starch used for the preparation of the suspension is preferably natural starch such as starch from maize, rice, tapioca, potato having a amylopectin content from 30 to 100%. Particularly prefered is maize starch, widely available on the market, having a typical amylopectin content of from 64-80% by weight. Within the scope of the invention, starch with a high content of amylose, such as amylomaize and chemically or physically modified starch can be used.

The starch suspension can also contain additives such as salts (e.g. saline coagulating agents as described in US Patent No. 4,853,168) alkaline agents, organic fillers or minerals, crosslinking agents, plasticisers, polyoxyethylene, polyvinyl alcohol, ionomeric polymers such as copolymers of ethylene and acrylic acid and/or maleic anhydride, polyacrylates, polyamides, lubricants such as lecithin, fatty acids, esters and amides of fatty acids.

The suspension, maintained in the disperser under stirring at ambient temperature, is then pumped via a gear pump 2 into a jet cooker, itself indicated with 3, where it is mixed in a cocurrent with steam in such a way as to reach the desired cooking temperature. The jet cooking process is known per se and involves instantaneous heating of the aqueous suspension with process steam and then maintaining the heated liquid for a predetermined period. The cooking temperature, generally between 90 and 180°C, is selected according to the specific starch used in the course of the process. In particular, care should be taken to avoid an excessively high temperature causing degradation of the starch material, while ensuring that the temperature, the shearing time applied and the standing time are such that it is possible to obtain a dispersion close to complete gelation.

At the outlet of the jet cooker, the starch dispersion or solution subject to cooking is collected whilst stirring in a lined stirred reactor 4, water circulating at a temperature of about 100°C in the casing thereof. A flash is effected in this lined tank in order to free the excess steam and to return the starch/water concentrations close to the initial concentrations.

From reactor 4 the starch is pumped via a pump 5, in a heat exchanger 6 where it is brought to a temperature of between 20 and 100°C, preferably from 40 to 70°C. From the heat exchanger, the starch is fed to a fibre making device of the types illustrated in figures 2 and 3, described in the following, in which a saline coagulating solution is also injected. The salts that can be used in the scope of the present invention comprise ammonium sulphate, magnesium sulphate, aluminium sulphate, ammonium phosphate, potassium chloride, sodium sulphate, sodium carbonate, sodium bicarbonate, and ammonium chloride. The preferred saline solution is a saturated solution of ammonium sulphate, although it is not necessary to reach saturated levels of the above mentioned salts and it is equally possible to use concentrations lower than saturation levels.

The starch fibres obtained from the fibre making device are collected in a stirred reactor 8 in order to be subjected to maturing and subsequently decanting. Once the decanting has been effected the clarified substance is recycled, by means of a pump 9, and mixed with a saturated saline solution of the coagulating agent before being reused for drawing the starch.

The clarified substance which circulates in the installation as a coagulating agent, contains the saline solution and the finest fibres which, due to their small dimensions are not decanted in the collecting container.

The mass of fibres from reactor 8 is pumped by means of pump 10 on to filter 11. The fibres are then collected in a container 12, while the filtrate is fed to container 13 where it is mixed with the clarified substance from pump 9, with subsequent addition of sulphate in order to recycle the saline solution adapted to be fed into fibre making device 7.

By using an appropriate number of reactors 8 for the maturing and decanting, it is possible for the process to be carried out continuously, thereby obtaining starch fibres which can be washed directly on the filter or simply filtered and subsequently washed.

The fibre making device 7, in the embodiement in figure 2, comprises a tubular body 14 having at least one inlet 15 which, under normal conditions, is used for feeding the starch material, an inlet 16 designed to feed the coagulating agent and a outlet 17 for discharging the starch fibres produced after the coagulation.

From the inlet 15 the starch material is immersed in a tubular duct 18 which partially terminates in a wall 19 supplied with radial holes. The holey wall part 19 acts as the distributor of the starch material flow towards a feeding chamber 21.

With the reference 22, the tubular element with microporous walls suitable for extruding the starch material from the feeding chamber 21 into the annular chamber 23 coaxially thereto is indicated. The chamber 23 is separated from the radially external surface of the element 22 and the radially internal surface of body 14.

The tubular element 22 can consist of a body of porous sintered metal material in which the distribution of the porous dimension is preferably comprised between 10 and 500 microns.

Alternatively the tubular element 22 is a body of metal material, for example stainless steel, provided with a number of radially passing holes obtained by mechanical working and having at least a narrow flow section with openings having a dimension preferably comprised between 10 and 500 microns. Preferably said radial holes have a cross section as illustrated in figure 4 with a portion 24 of the inlet for the starch material having a narrow opening, typically from 10 to 500 microns, and a portion 25 on the outlet of the starch material with an larger size opening, preferably comprised between 0.5 and 1.5 mm.

The opening density on the extrusion surface (intended as the surface of the tubular element in contact with the coagulating agent), expressed as a ratio of number of holes to surface area is preferably comprised between 4 and 0.05 holes/mm².

The coagulating agent fed through the inlet opening 16, flows through the annular element 26 having a crown of axial holes 27, acting as distributor, and is fed into the first annular chamber 28 defined by the walls 14 of the fibre making device and a tubular element coaxial to the body 29. From chamber 28 the flow is fed into the annular chamber of outlet 23, parallel to the radially external surface of the microporous tubular element 22, where the flow of coagulating agent interacts with the extrusion flow of the starch material.

The starch material is extruded in the form of a variety of threads which surround the extrusion surface in the guise of a tubular film.

Preferably the flow speed of the saline coagulating agent in the annular section of the outlet chamber 23 is maintained between 1 and 15 m/s.

The drawing ratio, intended as ratio of flow speed of the coagulating agent in the annular section of the chamber 23 and the speed of the starch material at the outlet of the holes of the microporous wall (defined as the ratio between the flow rate of the starch material and the total section in the holes of the outlet) is generally comprised between 1-1000, preferably between 100-1000. Preferably the axial length of the outlet chamber 23 is such that a stay time of the starch material comprised between 5 and 15 milliseconds is obtained. In any case the axial length of the chamber 23 in which the starch material undergoes drawing must be such to cause an orientation of the starch material allowing at the same time a complete phase inversion.

At the outlet of chamber 23 the extruded flow is fed into a annular chamber 30 at a progressively increasing cross section in the flow direction.

In the embodiment of the fibre making device illustrated in figure 3, the flow of starch materials is fed through an inlet 31 to an annular chamber 32 defined by the walls of body 14 and the microporous walled tubular element 33. The flow of the starch material follows the radial direction towards the inside through the walls of element 33 into the annular outlet chamber 34 comprised between the tubular element 33 and a central nucleus 35 coaxial to the body. The flow of the coagulating agent is fed across an inlet 36 and into a prechamber 37, it flows into a chamber 40 across holes 39 of an annular element 38 and from chamber 40 is fed to the outlet chamber 34 having a narrow cross section in the flow direction.

In this embodiment the section of holes of the microporous element 33 remains the same as figure 4. In this case, however, the flow of the starch material advances from a bigger to a smaller cross section, which brings an increase in the starch flow speed and necking down of the starch threads. The material leaving the holes is coagulated by the coagulation agent flow in the annular chamber 34. It has been observed that the best conditions of coagulation are when the drawing ratio is comprised preferably between 1 and 150, with an emission speed of the starch material from the holes in the microporous walls 33 comprises preferably between 0.1 and 1 m/s.

The fibre making device subject of the present invention presents notable advantages such as:
- it supplies, through coagulation of a starch material, a product having a fibrous structure;
- its structure having a cylindrical symmetry guarantees uniformity of fluid mechanic conditions thus excluding possible border effects;
- its geometry is completely known and therefore project criteria are available.
- the knowledge of the above mentioned criteria permits its scale-up.

Other advantages deriving from the use of the above fibre making device, will be highlighted by the following examples.

### Example 1

By using a plant as described with reference to figure 1 maize starch fibres have been obtained working under the following conditions:
- starch concentration in the dispersion : 15% by weight (anhydrous starch)
- maximum cooking temperature in the jet cooker: 115°C (preferred temperature range is between 100-130°C)
- temperature of the starch at the inlet of the fibre making device: 60°C
- saline solution: ammonium sulphate: 41% by weight
- temperature of the saline solution at the fibre making device inlet: 21°C
- maximum speed of the saline solution in the outlet chamber of the fibre making device: 7 m/s
- flow rate of the starch after cooking 48 l/h
- fibre making device as illustrated in figure 2 having a extrusion sinter consisting of a sintered metal with a porosity of 40 microns (average diameter of the pores)
- length of the outlet chamber (23,24) of the fibre making device: 10 cm
- average maturing time before filtering : 4 hours

Carrying out the process according to the above mentioned conditions starch fibres were obtained having the following size distribution measured according to the Bauer McNett apparatus expressed in percent by weight:

| | |
|---|---|
| 595 µm (28 mesh)% | 0.3 |
| 297 µm (40 mesh)% | 3.1 |
| 149 µm (100 mesh)% | 68.5 |
| 74 µm (200 mesh)% | 21.3 |
| above 200 mesh X 100 | 6.8 |

The determination of the characteristics of the solubility and the fibre obtained has been carried out using the following procedure:
washing of the filtration panels coming from the plant; 100 g of the filtration cake are dispersed in water (500 ml) by mechanical stirring with a glass anchor stirrer under the following conditions:
Becker with diameter 10 cm and height 20 cm; mechanical glass anchor stirrer (1=40 cm with stirring blade with 1= 8 cm, height 8 cm);
Temperature = 20°C; stirring time 30 mins; rotation speed 500 rpm.

The dispersion obtained is filtered on Bruckner with a diameter of 30 cm in the presence of a paper filter under vacuum of 10 mm Hg.

The liquid is filtered twice on the same panel. The panel is then washed with 500 ml of H₂O. The ratio of starch to water in the washing is 1:10.

The solubility determination is carried out on the filtered product, in order to separate it from the water and washed to remove the coagulant. The product is dispersed in water in a conventional laboratory pulper (dry concentration 0.2% rotation speed 3000 rpm); a sample was removed after 4 hours and after filtered on a 8 micron filter paper, the starch is measured in solution with the reagent "ANTHRONE" (solution 0.2% of ANTHRONE in 96% H₂SO₄).

The solubility value, determined by the above cited method on the filter panels obtained according to the example, is less than 1.5%.

The morphological characteristics of the fibre obtained are illustrated in figure 4.

### Example 2

The test according to example 1 has been repeated varying only the characteristics of the microporous sintered filter consisted, in this case of a sintered metal tube with pores having an average diameter of 100 µm. Fibres were obtained having the following size distribution expressed in terms of percentage by weight:

| | |
|---|---|
| 595 µm (28 mesh)% : | 0.3 |
| 297 µm (40 mesh)% : | 0.9 |
| 149 µm (100 mesh)% : | 63 |
| 74 µm (200 mesh)% : | 25.2 |
| above 200 mesh X 100 : | 10.6 |

The results demonstrate that the average diameter of the pores does not influence in a relevant way the fibre distribution that is maintained on a 100 and 200 mesh.

The solubility values obtained according to the method of example 1 are once again less than 1.5% like in the preceding case.

### Example 3 (comparative)

The characteristics of the fibres obtained by the test in example 1 are compared to the fibrids obtained with the other fibre making devices, in particular ejector and spinneret.

The process conditions are the same as for example 1.

The first fibre making device consists of an ejector equipped with 8 holes in a 1 mm diameter, for the starch inlet with an inclination of 45° with respect to ejector axis placed in the groove. The speed of the coagulating agent (ammonium sulphate) in the thinner section is equal to 31 m/s and the draw ratio, (defined as the ratio between the maximum speed of the sulphate to that of the starch leaving the holes) is equal to 47.

The second fibre making device consists of a spinneret equipped with 113 holes having a diameter of 0.5mm; this spinneret is placed in a circular duct and the annular crown separated from the external surface of the spinneret and the internal walls of the circular duct is fed with the coagulating agent, ammonium sulphate: the speed of the ammonium sulphate and that of the starch material exiting the holes are parallel. At the holes outlet, the starch material is contacted with the coagulating agent; the suspension formed then enters in a convergent (having a minimum diameter of 4 mm which corresponds to a sulphate speed of 30 m/s) in which the high turbulence completes the coagulation.

Table 1 reports the comparison of the fibre distribution for the various products; as can be noted, with the ejection fibres there is a high percentage of fine particles (80%) which reduces when passing to the spinneret and the tubular. The distribution curve is also different for these two fibre making device: very narrow for the tubular (90% of the particles between 100 and 200 mesh), larger for the spinneret.

This size distribution, combined with the particle form (similar to fibres with a marked form ratio such as for tubular; with high film content, furled and without a preferred direction in the case of the spinneret) is responsible for the different behaviour of the two products in the paper preparation together with the cellulose fibres. In fact it has been experimentally verified that the products obtained from the tubular fibre making device does not give rise to problems (of moulding or desiccation) in the preparation of sheets in the laboratory while the use of the product from the spinneret, starting from a certain percentage, gives sheets with surface defects and with a tendency to stick to the sheet forming plate.

Table 2 reports the percentage of starch retained on the sheet of paper prepared in the laboratory with the Rapid-Koethen apparatus, after dispersion of the cellulose - starch material paste (at 10 % of the latter) in the pulper for 2 hours at 3000 rpm at ambient temperature. As noted the highest retention is with the product from the tubular fibre making device.

Table 3 finally highlights the behaviour of the two different products when filtered from the slurry after the coagulation and washing until the ammonium sulphate has been eliminated, the concentrations of the slurry and the maturing time being equal. As shown the products obtained from the tubular fibre making device show a double productivity with respect to those of the spinneret.

Moreover another subject of the present invention are the starch fibres obtainable through the previously described method that present the characteristic of having a solubility of less than 2% and a dimension distribution as such of 90% has a dimension such as to enter in the range of from 100 to 200 mesh, after classification by the Bauer-McNett apparatus.

**Table 1-**

| SRC Distribution with various fibre making devices | | | | | |
|---|---|---|---|---|---|
| Fibre making device | Distribution (% w/w) | | | | |
| | 28 | 50 | 100 | 200 | >200 |
| spinneret | 0.1 | 7.6 | 35.3 | 31.0 | 26 |
| ejector | 0.3 | 0.4 | 4.2 | 14.6 | 80.5 |
| tubular | 0.3 | 3.1 | 68.5 | 21.3 | 6.8 |

**Table 2 -**

| Retention of starch fibres/fibrids in the paper | |
|---|---|
| Fibre making device | Retention % |
| Spinneret | 87.5 |
| Ejector | 77 |
| Tubular | >99 |

**Table 3 -**

| Filtering capacity of various starch fibres/fibrids | |
|---|---|
| Fibre making device | Filtered solid (Kg/h) |
| tubular | 20 |
| spinneret | 10 |

## Claims

1. A process for the preparation of fibres of starch material which comprises preparing an aqueous dispersion or solution of starch material and extruding this into a solution of a saline coagulating agent characterised in that the aqueous dispersion or solution of starch material is extruded through a microporous tubular wall of a chamber circularly ringed with said microporous wall into an annular chamber through which the solution of coagulating agent is caused to flow whereby the contact of the flowing coagulating agent solution with the extruded starch material dispersion or solution coagulates the starch material to form a fibrous structure.

2. A process according to claim 1, wherein the aqueous dispersion or solution of starch material is extruded through a microporous wall which presents holes having at least a section with an average diameter comprised between 10 and 500 microns and which has a density of extrusion surface holes comprised between 4 and 0.05 holes/mm².

3. A process according to claim 2, in which the aqueous dispersion or solution of starch material is extruded through a microporous tubular wall having a narrow inlet section and having an opening size of from 10 to 500 microns in to a larger outlet having an opening size greater than the said narrow section and wherein the drawing ratio is comprised between 100 and 1000.

4. A process according to claim 2, in which the aqueous dispersion or solution of starch material is extruded through a micrporous tubular wall having a narrow inlet section and having an opening size of from 10 to 500 microns and less than the size of opening of said larger section and wherein the drawing ratio is comprised between 1 and 150.

5. A process according to any one of the previous claims 1 to 4, in which the standing time of the starch material in said annular chamber is comprised between 5 and 15 milliseconds.

6. A fibre making device, particularly for the production of starch fibres through extrusion of a flow of starch material in a flow of coagulating agent characterised in that it comprises:
- a tubular body (14) comprising first means of entry (15,31) for feeding the flux of starch material.
- a feeding chamber for the starch material (21, 32) connection the said first means of entry,
- an annular outlet chamber (23, 34) of the starch material,
- a tubular element (22, 33) with porous walls coaxially arranged with said outlet chamber (23, 34) and interposed between the latter and the feeding chamber (21, 32), adapted to extrude through the said porous walls in said outlet chamber a variety of threads of starch material,
- a second means of entry (16, 36) connecting the said outlet chamber for feeding a coagulating agent flow,
and
- means of discharge (17, 30) arranged downstream from and connected to the annular outlet chamber.

7. A fibre making device according to claim 6 characterised in that said tubular element with porous wall (22, 33) is constituted of a sintered metal having pores with a distribution comprised between 10 and 500 microns.

8. Fibre making device according to claim 6 characterised in that said tubular element (22, 33) with microporous wall is a cylindrical element with holey walls having a plurality of radially passing holes (24, 25) having at least one narrow section with a dimension comprised between 10 and 500 microns.

9. Device according to claim 7 or 8 in which said pores present an area density on the extrusion surface of from 4 to 0.05 holes/mm².

10. Fibre making device according to claim 8 in which said annular outlet chamber (23) of the starch material is coaxial and radially external to said feeding chamber (21).

11. Device according to claim 10 in which said radial holes comprise a section (24) connecting with the feeding chamber (21) having a size of opening comprised between 10 and 500 microns and a section (25) connecting with the said outlet chamber having the size of opening larger to the size of opening of said section (24).

12. Device according to claim 8 in which said annular outlet chamber (34) is coaxial and radially internal to the said feeding chamber (32).

13. Device according to claim 12 in which said radial holes comprise a section (24) connecting with the outlet chamber (34) having a size of opening comprised between 10 and 500 microns and a section (25) connecting with the feeding chamber (32) having a size of opening larger to the size of opening of said section (24).

14. Starch fibres obtained through a process according to any of the claims 1 to 5 having a solubility of less than 2% and size distribution such for which 90% of the fibres have a dimension such as to enter in the range of from 100 to 200 mesh, after classification by the Bauer-McNett apparatus.

## Patentansprüche

1. Verfahren zur Herstellung von Fasern aus Stärkematerial, das umfaßt, daß man eine wäßrige Dispersion oder Lösung von Stärkematerial herstellt und diese in eine Lösung eines kochsalzhaltigen koagulierenden Mittels extrudiert, dadurch gekennzeichnet, daß man die wäßrige Dispersion oder Lösung des Stärkematerials durch eine mikroporöse rohrförmige Wand einer Kammer, die ringförmig von der mikroporösen Wand umgeben ist, in eine ringförmige Kammer extrudiert, durch die die Lösung des koagulierenden Mittels strömen gelassen wird, wodurch der Kontakt der strömenden Koagulierungsmittellösung mit der extrudierten Stärkematerialdispersion oder Lösung das Stärkematerial unter Bildung einer faserigen Struktur koaguliert.

2. Verfahren nach Anspruch 1, worin die wäßrige Dispersion oder Lösung des Stärkematerials durch eine mikroporöse Wand extrudiert wird, die Löcher aufweist, mit mindestens einem Abschnitt mit einem durchschnittlichen Durchmesser zwischen 10 und 500 µm, der eine Dichte von Extrusionsoberflächenlöchern zwischen 4 und 0,05 Löchern/mm² aufweist.

3. Verfahren nach Anspruch 2, worin die wäßrige Dispersion oder Lösung des Stärkematerials durch eine mikroporöse rohrförmige Wand mit einem schmalen Einlaßabschnitt und einer Öffnungsgröße von 10 bis 500 um zu einem größeren Auslaß mit einer Öffnungsgröße, die größer ist als die des schmalen Abschnitts, extrudiert, wobei das Reckverhältnis zwischen 100 und 1000 liegt.

4. Verfahren nach Anspruch 2, worin die wäßrige Dispersion oder Lösung des Stärkematerials durch eine mikroporöse röhrenförmige Wand extrudiert wird mit einem schmalen Einlaßbereich und einer Öffnungsgröße von 10 bis 500 µm, der kleiner ist als die Größe der Öffnung des größeren Bereichs, wobei das Reckverhältnis zwischen 1 und 150 liegt.

5. Verfahren nach einem der vorhergehenden Ansprüche 1 bis 4, worin die Standzeit des Stärkematerials in der ringförmigen Kammer zwischen 5 und 15 ms liegt.

6. Faserherstellungsvorrichtung, insbesondere zur Herstellung von Stärkefasern durch Extrusion einer Stärkematerialströmung in einen Strom eines Koagulierungsmittels, dadurch gekennzeichnet, daß sie:
- einen röhrenförmigen Körper (14) mit einer ersten Eintrittseinrichtung (15, 31) zur Zuführung des Stroms aus Stärkematerial
- eine Beschickungskammer für das Stärkematerial (21, 32) in Verbindung mit der ersten Eintrittseinrichtung,
- eine ringförmige Auslaßkammer (23, 34) für das Stärkematerial
- ein Röhrenelement (22, 33) mit porösen Wänden, das koaxial zu der Auslaßkammer (23, 34) angeordnet ist und zwischen die letztere und die Beschickungskammer (21, 32) zwischengeschaltet ist, das so ausgebildet ist, daß durch die porösen Wände in der Auslaßkammer eine Vielzahl von Fäden aus Stärkematerial extrudiert werden
- eine zweite Eintrittseinrichtung (16, 36) in Verbindung mit der Auslaßkammer zur Beschickung mit einer Koagulationsmittelströmung und
- eine Austragseinrichtung (17, 30), die stromabwärts der ringförmigen Auslaßkammer angeordnet ist und mit ihr verbunden ist, umfaßt.

7. Faserherstellungsvorrichtung nach Anspruch 6, dadurch gekennzeichnet, daß das Röhrenelement mit poröser Wand (22, 33) aus einem gesinterten Metall mit Poren mit einer Verteilung zwischen 10 und 500 um gebildet wird.

8. Faserherstellungsvorrichtung nach Anspruch 6, dadurch gekennzeichnet, daß das Röhrenelement (22, 33) mit mikroporöser Wand ein zylindrisches Element mit löchrigen Wänden mit einer Vielzahl von radial hindurchgehenden Löchern (24, 25) ist, das mindestens einen engen Bereich mit einer Dimension zwischen 10 und 500 um aufweist.

9. Vorrichtung nach Anspruch 7 oder 8, worin die Poren in einer Flächendichte auf der Extrusionsoberfläche von 4 bis 0,05 Löchern/mm² vorhanden sind.

10. Faserherstellungsvorrichtung nach Anspruch 8, worin die ringförmige Auslaßkammer (23) des Stärkematerials koaxial zu der Beschickungskammer (21) und radial außerhalb davon ist.

11. Vorrichtung nach Anspruch 10, worin die radialen Löcher einen Abschnitt (24), der mit der Beschickungskammer (21) verbunden ist, mit einer Öffnungsgröße, die zwischen 10 und 500 µm liegt, und einen Bereich (25), der mit der äußeren Kammer verbunden ist, mit einer Öffnungsgröße, die größer ist als die Größe der Öffnung des Abschnitts (24), umfassen.

12. Vorrichtung nach Anspruch 8, worin die ringförmige Auslaßkammer (34) koaxial zu der Beschickungskammer (32) und radial innenliegend ist.

13. Vorrichtung nach Anspruch 12, worin die radialen Löcher einen Abschnitt (24), der mit der Auslaßkammer (34) verbunden ist, mit einer Öffnungsgröße, die zwischen 10 und 500 µm liegt, und einen Abschnitt (25), der mit der Beschickungskammer (32) verbunden ist, mit einer Öffnungsgröße, die größer ist als die Öffnungsgröße des Abschnitts (24), umfassen.

14. Stärkefasern erhalten mit einem Verfahren nach einem der Ansprüche 1 bis 5 mit einer Löslichkeit von weniger als 2% und einer solchen Größenverteilung, daß 90% der Fasern eine solche Dimension haben, daß sie in dem Bereich von 100 bis 200 mesh liegen nach einer Klassierung mit der Bauer-McNett-Vorrichtung.

## Revendications

1. Procédé pour la préparation de fibres d'une matière de type ou à base d'amidon ou de fécule, ce procédé comprenant la préparation d'une dispersion ou solution aqueuse d'amidon ou de fécule et l'extrusion de cette dispersion ou solution dans une solution d'un agent salin de coagulation, procédé caractérisé en ce que la dispersion ou solution aqueuse de la matière du type ou à base d'amidon ou de fécule est extrudée à travers une paroi tubulaire microporeuse d'une chambre entourée circulairement par ladite paroi microporeuse dans une chambre annulaire à travers laquelle la solution de l'agent de coagulation est obligée de s'écouler, de sorte que le contact de la solution d'agent de coagulation en circulation avec la dispersion ou solution de la matière de type ou à base d'amidon ou de fécule extrudée coagule la matière de type ou à base d'amidon ou de fécule pour former une structure fibreuse.

2. Procédé selon la revendication 1, dans lequel la dispersion ou solution aqueuse de la matière à base ou du type amidon ou fécule est extrudée à travers une paroi microporeuse qui présente des trous ayant au moins une section d'un diamètre moyen compris entre 10 500 micromètres, et qui a une densité de trou(s) dans la surface d'extrusion comprise entre 4 et 0,05 trou/mm².

3. Procédé selon la revendication 2, dans lequel la dispersion ou solution aqueuse de matière de type ou à base d'amidon ou de fécule est extrudée à travers une paroi tubulaire microporeuse ayant une section d'entrée étroite et ayant une taille d'ouverture de 10 à 500 micromètres dans une sortie plus large ayant une taille d'ouverture ou une lumière supérieure à ladite section étroite, le rapport ou taux d'étirage étant compris entre 100 et 1000.

4. Procédé selon la revendication 2, dans lequel la solution ou dispersion aqueuse de matière de type ou à base d'amidon ou de fécule est extrudée à travers une paroi tubulaire microporeuse ayant une section d'entrée étroite et ayant une taille d'ouverture ou lumière de 10 à 500 micromètres et qui est inférieure à la taille d'ouverture de ladite section plus grande, procédé dans lequel le rapport ou taux d'étirage est compris entre 1 et 150.

5. Procédé selon l'une quelconque des revendications 1 à 4 précédentes, dans lequel le temps de séjour de la matière de type ou à base d'amidon ou de fécule dans ladite chambre annulaire est compris entre 5 et 15 millisecondes.

6. Dispositif de production de fibres, en particulier pour la production de fibres d'amidon ou de fécule par extrusion d'un courant de matière de type ou à base d'amidon ou de fécule dans un agent coagulant en écoulement, dispositif caractérisé en ce qu'il comprend:
- un corps tubulaire (14) comprenant un premier moyen d'entrée (15, 31) pour l'introduction du flux de la matière de type ou à base d'amidon ou de fécule;
- une chambre d'alimentation en la matière de type ou à base d'amidon ou de fécule (21, 32) connectée audit premier moyen d'entrée;
- une chambre annulaire de sortie (23, 34) de la matière du type ou à base d'amidon ou de fécule;
- un élément tubulaire (22, 33) comportant des parois poreuses disposées coaxialement avec ladite chambre de sortie (23, 34) et interposé entre cette chambre et la chambre d'alimentation (21, 32), cet élément convenant pour une extrusion à travers lesdites parois poreuses dans ladite chambre de sortie de divers fils de matière à base d'amidon ou de fécule;
- un second moyen d'entrée (16, 36) reliant ladite chambre de sortie pour introduire un courant d'agent de coagulation; et
- un moyen de décharge (17, 30) disposé en aval de la chambre annulaire de sortie et relié à cette chambre.

7. Dispositif de production de fibres selon la revendication 6, caractérisé en ce que ledit élément tubulaire comportant une paroi poreuse (22, 33) est constitué d'un métal fritté ayant des pores présentant une distribution des tailles comprise entre 10 et 500 micromètres.

8. Dispositif de fabrication de fibres selon la revendication 6, caractérisé en ce que ledit élément tubulaire (22, 33) comportant une paroi microporeuse est un élément cylindrique présentant des parois foraminées ayant plusieurs trous (24, 25) passant radialement et ayant au moins une section étroite de dimension comprise entre 10 et 500 micromètres.

9. Dispositif selon la revendication 7 ou 8, dans lequel lesdits pores présentent, par rapport à la surface d'extrusion, une densité surfacique de 4 à 0,05 trou/mm².

10. Dispositif de fabrication de fibres selon la revendication 8, dans lequel ladite chambre annulaire de sortie (23) de la matière de type ou à base d'amidon ou de fécule est coaxiale et radialement externe par rapport à ladite chambre d'alimentation (21).

11. Dispositif selon la revendication 10, dans lequel lesdits trous radiaux comprennent un tronçon ou une section (24) en liaison avec la chambre d'alimentation (21), ayant une taille d'ouverture ou lumière comprise entre 10 et 500 micromètres et un tronçon ou section (25) de liaison avec ladite chambre de sortie ayant une taille d'ouverture ou lumière plus grande que la taille de l'ouverture de ladite section ou dudit tronçon (24).

12. Dispositif selon la revendication 8, dans lequel ladite chambre annulaire (34) de sortie est coaxiale et radialement intérieure par rapport à ladite chambre (32) d'alimentation.

13. Dispositif selon la revendication 12, dans lequel lesdits trous radiaux comprennent un tronçon ou une section (24) de liaison avec la chambre de sortie (34) ayant une taille d'ouverture ou lumière comprise entre 10 et 500 micromètres et un tronçon ou section (25) de liaison avec la chambre d'alimentation (32) ayant une taille d'ouverture ou lumière plus grande que la taille d'ouverture de ladite section ou dudit tronçon (24).

14. Fibres de fécule ou d'amidon, obtenues à l'aide d'un procédé selon l'une quelconque des revendications 1 à 5, ayant une solubilité inférieure à 2% et une distribution de taille telle que 90% des fibres ont une dimension leur permettant de pénétrer dans les mailles d'une toile de tamis numéro 100 à 200, après classification par l'appareil de Bauer-McNett.
